

# UNITED STATES PATENT OFFICE.

GEORGE BRINTON FRALEY, OF PHILADELPHIA, PENNSYLVANIA, ASSIGNOR,  
BY MESNE ASSIGNMENTS, TO OSCAR A. FOW AND DAVID W. VAN TINE,  
OF SAME PLACE.

## COMPOSITION OF MATTER FOR ELECTRIC HEATERS.

SPECIFICATION forming part of Letters Patent No. 606,921, dated July 5, 1898.

Application filed August 12, 1897. Serial No. 647,988. (No specimens.)

*To all whom it may concern:*

Be it known that I, GEORGE BRINTON FRALEY, a citizen of the United States, residing in the city and county of Philadelphia, State 5 of Pennsylvania, have invented a new and useful Improvement in Composition of Matter for Electric Heaters, which improvement is fully set forth in the following specification.

In carrying out my invention I take talc, 10 say sixty parts; silicate of soda, say twenty parts; carbonate of soda, say ten parts; water, say ten parts, and thoroughly mix the same, producing a mass which when set may be

heated by electric wires or conductors placed therein or thereon, while being non-conductors of electricity. 15

What I claim, and desire to secure by Letters Patent, is—

A composition of matter consisting of talc, silicate of soda, carbonate of soda, and water 20 in substantially the proportions set forth.

GEORGE BRINTON FRALEY.

Witnesses:

JOHN A. WIEDERSHEIM,  
WM. C. WIEDERSHEIM.

O'Neill, 498,078, Stoves & Furnaces, Elec. Heaters,

Kester, 524,062, Aug. 7, 1894, " "